

April 14, 1953

A. B. BAGSAR  
MONOLITHIC METAL STRUCTURE

2,634,699

Filed Nov. 20, 1948



FIG. 2.



FIG. 1.



FIG. 3.



FIG. 4.

INVENTOR.  
AARON B. BAGSAR  
BY  
*Busser and Harding*  
ATTORNEYS

## UNITED STATES PATENT OFFICE

2,634,699

## MONOLITHIC METAL STRUCTURE

Aaron B. Baggas, Drexel Hill, Pa., assignor to Sun  
Oil Company, Philadelphia, Pa., a corporation  
of New Jersey

Application November 20, 1948, Serial No. 61,255

4 Claims. (Cl. 114—79)

1

The development of fusion welding has resulted in its successful application to various monolithic steel constructions. An early application was to structures such as pressure vessels, after which the shipbuilding industry adopted this method of construction as a substitute for the riveted type of construction. The welding method has also been applied to a certain extent to bridges and other massive structures.

The known advantages of the welded over the riveted construction include: considerable weight- and material-saving effected by eliminating lapped seams; appreciably stronger seams obtained by welding, since the riveted construction requires drilling or punching through the structural members; no maintenance problems involved similar to riveted seams, such as leaks occurring through rivet holes due to corrosion or excessive flexing, etc., obtaining a flush job, thereby simplifying internal drainage and painting problems and obtaining a stream-line construction, thereby reducing frictional loss.

However, in certain all-welded constructions of monolithic type, certain difficulties have developed that were not foreseen and which in some cases have had serious consequences, such difficulties being characteristic of those monolithic steel structures which are subject to multiaxial and severe stresses. For example, in ship construction serious fractures were encountered, because a normally ductile steel would exhibit a brittle fracture in a welded ship, due to complexity of the stresses imposed by construction and by the service conditions, these fractures mostly occurring in the plates and not in the weld itself. In order to minimize these difficulties it was later proposed to insert in certain critical sections riveted seams in order to break up the continuity of the plates in the welded structures and also to obtain a certain amount of flexing, the purpose being to at least arrest the extent of cracking. It has also been proposed to add numerous structural members to the ship's structure, mainly internally, in order to relieve the welded shell of the ship from excessive stresses, with the object of thereby preventing cracking of the hull and decking.

Both the above remedies have distinct limitations and disadvantages. They may reduce, but do not eliminate, the danger of losing a ship by fracturing of the hull.

Insertion of riveted seams in critical sections of the ship is distinctly objectionable, since riveting requires drilling of the main shell at these sections in order to install rivets, thereby seriously

reducing the strength of the section. This modification is also objectionable for the reason that most of the stresses are thrown onto these riveted seams, because the remainder of the shell and decking is continuous by virtue of the fact that the plates are welded together and do not therefore flex as much as the riveted joint. Still another objection to this expedient is that the rivets in these insertions leak badly after a short service; which may be due to the excessive flexing and stressing that are induced in these seams, since the remainder of the shell is welded and continuous. These stresses are therefore more severe than in a wholly riveted shell, since in the latter such stresses are more evenly distributed over a number of riveted joints.

The insertion of independent members in the ship to stiffen the ship's structure is also objectionable because of the difficulty of installing the sections in such a manner and with such rigidity as to make these additional sections share proportionately the stress simultaneously with the remaining members of the ship's structure. In the circumstances, the hull fails first before the stress is transmitted to these additional stiffeners, or in other cases the stiffeners fail first and transmit the stress to the ship's shell, thereby rendering the stiffeners ineffective.

It is known that riveted seams are not as susceptible to crack propagation as welded ships of monolithic type, and that cracks may be arrested in these riveted seams, although failure of riveted seams themselves by cracking is not altogether uncommon. It is believed that the virtue of the riveted seam in this respect over the welded construction is attributable to the fact that no excessive stress concentrations are possible because of the relative flexibility of the riveted seam, and also to the inherent geometry of the riveted seam in which the adjoining plates are not made integral with each other, as in welding, but are held together mechanically by rivets and butt straps or by the lapping arrangement.

In welded bridge and other massive constructions, also, similar defects exist and similar serious fracturing has resulted, which, in the opinion of some engineers, make the application to bridges and other massive structures of fusion welding impracticable, notwithstanding the recognized advantages of such type of construction. Even pressure vessels of the welded monolithic type, such as gas storage tanks, are not immune to the dangers above outlined, which are not satisfactorily remediable by any of the above specified

expedients that break up the continuity of the plates. In fact the application of butt-welding, as distinguished from riveting, to structural steel generally, notwithstanding its pronounced advantages over riveting, has been restricted and, in some proposed applications, prevented, by the special defects above set forth.

Regardless of all the care exercised to eliminate welding imperfections and to improve workmanship, some irregularities will be present in the completed welded construction, such as imperfect weld penetration, misalignment, inclusions in the welded seams, weld undercutting, and certain discontinuities in the steel plates themselves which are difficult to eliminate altogether, such as scratches, arc craters, segregations or laminations. The loci of such imperfections act as focal points from which cracks may start, and unless some means is provided to arrest them, these cracks will assume serious proportions. In the case of a ship a single crack may wholly incapacitate it or even cause it to break into sections.

The object of my invention is to arrest the extension of shearing or tearing fractures of local origin while avoiding the limitations and disadvantages of both the riveted and welded construction and of the expedients heretofore adopted having the same object. I have found that a metal plate composed of certain materials other than plain carbon steel (which is utilized in welded ship construction and in other structures of the welded monolithic type) and which, unlike plain carbon steel, will not become brittle and will maintain a high degree of ductility at low temperature, will effectively resist cracking or fracturing under stresses that will readily propagate a crack through carbon steel. A ship hull or deck composed entirely of plates of such material would effectively resist cracking or fracturing; but many of such compositions would be subject to deteriorating conditions to which steel is resistant and all of such compositions are so relatively expensive that, if they were equal to steel in all other respects, the cost would be prohibitive. I have discovered, however, that even when a single plate of such composition is applied to a monolithic welded steel plate structure, it will arrest, beyond its locus of application, the advance of any crack that is propagated through a contiguous multi-plate steel structure. Compositions suitable for such applied units are known to the metallurgist and are too numerous to detail; but as examples may be cited copper, brass, nickel-copper, and many alloy steels such as chromium steel, nickel steel and nickel-chromium steel. All these materials are characterized by a pronounced degree of ductility at temperatures as low as any that might be reasonably expected to be encountered by a ship, pressure vessel, storage tank, bridge, etc., or (say) any temperature down to or even below minus 50° F. At the above temperature, what is known as plain or ordinary carbon steel of commerce, composed almost or entirely of iron, carbon, manganese and silicon, disregarding an almost negligible quantity of impurities such as phosphorus and sulfur, has no measurable ductility, whether determined by elongation or bending tests, at a low temperature approaching minus 50° F.

Plates of this character may be inserted between the conventional steel plates and butt-welded thereto, or they may be applied to the interior or exterior face of the monolithic steel structure, and they may or may not be protected

from contact with water or other fluid to which they may be subjected by enclosing or overlapping plates of steel.

The invention may best be understood by reference to the following description of the attached drawings, in which—

Fig. 1 is a plan view of the deck of a ship.

Fig. 2 is a transverse vertical sectional view taken along the line 2—2 of Fig. 1 or along any transverse line across the area of the deck or hull desired to be protected.

Fig. 3 is a cross-sectional view of a special plate or strip interposed between and welded to adjacent conventional steel plates.

Fig. 4 is a cross-sectional view of another embodiment of the invention in which a special plate or strip is applied to one or more conventional steel plates.

In Figs. 1, 2 and 3, the plates marked *a* are conventional plates of carbon steel, while the plates or strips marked *b* are special units interposed between, and butt-welded to, the conventional plates. Each special unit is of a composition, other than carbon steel (which at low temperature becomes brittle and is non-resistant to cleavage fracture), that maintains its ductility at any temperature to which the ship hull might be exposed. There are a great number of metals that maintain their ductility, that is, are non-brittle, and hence are not subject to cleavage fracture, at a temperature below that specified, say, safely below minus 50° F., for example, copper, brass, or a nickel-copper alloy, or, in fact, many alloy steels, such as chromium steel, nickel steel, nickel-chromium steel and molybdenum bearing steels. Metallurgists well know that carbon steel loses its ductility when exposed to temperatures no lower than that which a ship normally encounters in service and they also know that there are various metal elements and metal alloys that retain their ductility no matter what low temperature it may be expected to encounter in service. If the entire hull of the ship were composed of plates having the ductility of said special units, as, for example, stainless steel, the danger of transverse cracking or fracturing would be obviated; but many of such substitute metals or alloys would not be suitable for various reasons, and any that would be suitable would be commercially impracticable, since the cost of such a construction would be prohibitive. I have found, however, that if the described special strips extend, as indicated in Fig. 1, longitudinally of the ship across the area desired to be protected, but occupying a very minor width of the hull and deck, the resistance to cracking or fracturing in the direction indicated by the arrow is effectual; that is, the crack will extend through a conventional plate or plates until it meets a special unit, when it encounters a barrier through and beyond which it cannot proceed. Such a crack or fracture usually starts at or near the angle between the hull and the deck, but wherever it starts it cannot extend entirely across the hull or deck.

While two long special strips *b* applied to the deck (if the deck is to be protected) and two long strips *b* applied to the hull afford adequate protection, it is desirable to apply additional long strips *c*, especially to the hull. It is not necessary, however, that each of the special units shall be a long strip extending entirely along the protected area. For such long special strips may be substituted, or to such long special strips may be added, a number of relatively short units, marked *d*, so

distributed (preferably staggered as indicated) as to extend along a plurality of parallel lines extending longitudinally of the ship's hull across the area to be protected and thus adapted to intersect any line extending transversely of the ship's hull within that area. While in Figs. 1 and 2 these short units are shown as applied only to the deck, the protection of the hull from cracking or fracturing is of primary importance. These short strips are not in these figures shown as applied to the hull in order to avoid the confused showing that would result from overlapping of full and broken lines.

It is practicable, also, to confine the strips of special metal between strips of steel, so that only steel is exposed at the interior and exterior surfaces of the hull or deck, but this specific modification is not claimed, but forms the subject matter of an application filed of even date here-with, Serial No. 61,256.

Instead of interposing such special units *b*, or *c*, or *d*, between the conventional plates and butt-welding them thereto, as shown in Fig. 3, special plates or strips *e* of the special composition above described may be applied to the face (either exterior or interior) of the hull and (or) deck and welded thereto as shown in Fig. 4. Such special plates or strips may be distributed as illustrated in Fig. 1 at *b*, *c* and *d* and as described in specifying the distribution of inserted special butt-welded strips or plates. These special plates may overlap adjacent conventional plates, but this is not necessary, nor in fact desirable, especially in the construction of new ships, since separate conventional plates, with the special units applied thereto, may be fabricated before they are welded in place.

These special units may be provided with holes or slots, as disclosed in my application filed July 31, 1947, Serial No. 765,007, but such a modification is unnecessary, since, if the special units are of a composition that maintains pronounced ductility at low temperatures, it is unnecessary for the special units to present edges, not fused to the shell, extending longitudinally of the body of the ship.

What I claim and desire to protect by Letters Patent is:

1. A construction for the shell of a ship comprising a multitude of plates of plain carbon steel and welded joints by means of which said plates are secured together to form a monolithic structure, in which shell cracks that may develop tend to extend in one general direction, namely, transverse to the longitudinal axis of the shell, said construction also comprising a number of special metal strips, of a composition other than plain carbon, that maintain ductility at a temperature substantially below that at which plain carbon steel loses its ductility, welds uniting said strips to certain of said plates of plain carbon steel, said strips extending longitudinally of the axis of the shell, and thus transverse to said general direction, along a plurality of spaced apart lines one or more of which intersect any line transverse to the longitudinal axis of the shell within the area of the shell designed to be protected, to thereby arrest, and prevent the extension of,

any crack that may spread in such general direction.

- 5 2. A construction as defined in claim 1 in which the special metal strips are of substantially the same thickness as the plates of plain carbon steel to which they are welded and are applied by insertion in the shell with their opposite faces substantially aligned with the opposite faces of plates of plain carbon steel adjacent thereto and which are butt-welded to said plates.
- 10 3. A construction as defined in claim 1 in which the plain carbon steel plates within the designed protected area are imperforate and in which the special strips welded to the shell are applied to one face of the shell.
- 15 4. A construction for the shell of a ship comprising a multitude of plates of plain carbon steel and welded joints by means of which said plates are secured together to form a monolithic structure, in which shell cracks that may develop tend to extend in one general direction, namely, transverse to the longitudinal axis of the shell, said construction also comprising a number of special metal strips, of a composition other than plain carbon steel, that maintain ductility at a temperature substantially below that at which plain carbon steel loses its ductility, welds uniting said strips to certain of said plates of plain carbon steel, said special strips extending longitudinally of the axis of the shell and thus transverse to said general direction, each longitudinal arrangement constituting a unit and each strip being of a length that is short relative to the length of that area of the shell that is designed to be protected from crack extension, adjacent sides of said strips spaced apart, said units being arranged along a number of lines, extending longitudinally of the axis of the shell, that are transversely spaced apart, said special units being of such length that they are transversely opposite spaces between special units extending along other lines and are also transversely opposite ends of such special units extending along other lines and are thus in staggered relation, whereby any line transverse to the longitudinal axis of the shell within such area designed to be protected intersects one or more special units and is thus adapted to arrest, and prevent extension of, any crack that may spread in such general direction.

40 50 AARON B. BAGSAR.

References Cited in the file of this patent

UNITED STATES PATENTS

| Number    | Name             | Date           |
|-----------|------------------|----------------|
| 1,290,091 | Cole             | Jan. 7, 1919   |
| 1,446,274 | Roberts          | Feb. 20, 1923  |
| 2,419,218 | Jannsen          | Apr. 22, 1947  |
| 2,460,893 | MacCutcheon, Jr. |                |
| 60        | et al.           | Feb. 8, 1949   |
| 2,481,614 | Redmond          | Sept. 13, 1949 |

FOREIGN PATENTS

| Number     | Country       | Date          |
|------------|---------------|---------------|
| 65 159,914 | Great Britain | 1921          |
| 464,280    | Germany       | Aug. 15, 1928 |